



US006379266B1

(12) **United States Patent**  
Ogg et al.

(10) **Patent No.:** US 6,379,266 B1  
(45) **Date of Patent:** Apr. 30, 2002

(54) **FOUR PIECE GOLF BALL**(75) Inventors: **Steven S. Ogg; Pijush K. Dewanjee**,  
both of Carlsbad, CA (US)(73) Assignee: **Callaway Golf Company**, Carlsbad,  
CA (US)(\*) Notice: Subject to any disclaimer, the term of this  
patent is extended or adjusted under 35  
U.S.C. 154(b) by 0 days.(21) Appl. No.: **09/527,381**(22) Filed: **Mar. 16, 2000**(51) Int. Cl.<sup>7</sup> ..... **A63B 37/02**(52) U.S. Cl. ..... **473/358; 473/357**(58) Field of Search ..... 473/356, 357,  
473/359, 360, 361, 362, 363, 364, 365,  
358(56) **References Cited**

## U.S. PATENT DOCUMENTS

|             |          |                            |
|-------------|----------|----------------------------|
| 2,153,409 A | 4/1939   | Bogoslawsky                |
| 2,973,800 A | 3/1961   | Muccino                    |
| 3,553,159 A | 1/1971   | Miller et al.              |
| 4,272,079 A | * 6/1981 | Nakade et al. .... 473/357 |
| 5,020,803 A | 6/1991   | Gendreau et al.            |
| 5,273,286 A | 12/1993  | Sun                        |
| 5,334,673 A | 8/1994   | Wu                         |

|             |           |                             |
|-------------|-----------|-----------------------------|
| 5,542,663 A | 8/1996    | Kato et al.                 |
| 5,674,137 A | 10/1997   | Maruko et al.               |
| 5,692,974 A | 12/1997   | Wu et al.                   |
| 5,713,801 A | 2/1998    | Aoyama                      |
| 5,716,293 A | 2/1998    | Yabuki et al.               |
| 5,752,888 A | 5/1998    | Maruko et al.               |
| 5,772,530 A | 6/1998    | Kato                        |
| 5,797,808 A | 8/1998    | Hayashi et al.              |
| 5,816,940 A | 10/1998   | Hayashi et al.              |
| 5,816,941 A | * 10/1998 | Hayashi et al. .... 473/359 |
| 5,816,942 A | 10/1998   | Hayashi et al.              |
| 5,836,831 A | 11/1998   | Stanton et al.              |
| 5,908,358 A | 6/1999    | Wu                          |
| 6,117,024 A | * 9/2000  | Dawanjee .... 473/365       |

\* cited by examiner

Primary Examiner—Mark S. Graham

Assistant Examiner—Racann Gorden

(74) Attorney, Agent, or Firm—Michael A. Catania

(57) **ABSTRACT**

A four-piece golf ball is disclosed herein. The golf ball has a core with an oxygen barrier boundary layer, a wound layer and a polyurethane cover. The core is preferably composed of polybutadiene material. The boundary layer is preferably composed of a blend of ionomers. The cover is preferably composed of a thermosetting polyurethane material. The golf ball has exceptional distance, exceptional feel and exceptional durability.

2 Claims, 1 Drawing Sheet





FIG. 2

**FOUR PIECE GOLF BALL****CROSS REFERENCES TO RELATED APPLICATIONS**

Not Applicable

**STATEMENT REGARDING FEDERALLY SPONSORED RESEARCH OR DEVELOPMENT**

Not Applicable

**BACKGROUND OF THE INVENTION**

## 1. Field of the Invention

The present invention relates to a multiple layer golf ball. More specifically, the present invention relates to a four-piece golf ball wherein the golf ball has a core, a boundary layer, a wound layer and a cover.

## 2. Description of the Related Art

Golf balls have evolved throughout the history of the game. The first type of golf balls were the "featherie", a leather sphere stuffed with wet, compressed feathers. The next innovation in golf balls was the gutta percha one piece golf ball. As early as the 1800's, golfers realized that gutta percha golf balls with indented surfaces flew better than those with smooth surfaces. Hand-hammered gutta-percha golf balls could be purchased at least by the 1860's, and golf balls with brambles (bumps rather than dents) were in style from the late 1800's to 1908. In 1908, an Englishman, William Taylor, received a patent for a golf ball with indentations (dimples) that flew better and more accurately than golf balls with brambles. A. G. Spalding & Bros., purchased the U.S. rights to the patent and introduced the GLORY ball featuring the TAYLOR dimples. Until the 1970s, the GLORY ball, and most other golf balls with dimples had 336 dimples of the same size using the same pattern, the ATTU pattern. The ATTU pattern was an octohedron pattern, split into eight concentric straight line rows, which was named after the main producer of molds for golf balls. The only innovation related to the surface of a golf ball during this sixty year period came from Albert Penfold who invented a mesh-pattern golf ball for Dunlop. This pattern was invented in 1912 and was accepted until the 1930's.

Golf balls with a wound layer appeared in the 1920's, and have been refined since that time. In the 1930's through the 1960's, the major innovations in golf balls related to core development. In the 1960's, the development of ionomer materials, particularly the brand SURLYN® from Du Pont, became the major innovation for golf balls into the 1980's. In the 1970's, dimple pattern innovations also appeared from the major golf ball manufacturers. In 1973, Titleist introduced an icosahedron pattern which divides the golf ball into twenty triangular regions. In the late 1980's and into the 1990's, three-piece solid golf balls, as opposed to three-piece wound, began to appear from the major golf ball manufacturers. These three-piece solid golf balls involved two thermoplastic layers covering a core.

Although not commercialized, several patents have disclosed four-piece golf balls. One example is Sun, U.S. Pat. No. 5,273,286 for a Multiple Concentric Section Golf Ball, which was filed in 1992. Sun discloses a golf ball with a solid inner core, a graphite intermediate core, a polybutadiene outer core and a cover composed of balata, ionomer or urethane materials.

Other examples are Hayashi et al., U.S. Pat. No. 5,816,940 for a Wound Golf Ball, which was originally filed in Japan in 1996, and Hayashi et al., U.S. Pat. No. 5,797,808

for a Wound Golf Ball which was originally filed in Japan in 1996. The Hayashi patents disclose a polybutadiene center core, a thermoplastic enclosure layer (preferably an elastomer), a wound layer and a cover composed of an inner layer and an outer layer with both cover layers composed of thermoplastic materials.

Yet another example is Maruko et al., U.S. Pat. No. 5,674,137 which was originally filed in Japan in 1994. Maruko discloses a golf ball with a liquid filled core, a wound layer over the core, and inner and outer cover layers composed of an ionomer material. The primary objective of Maruko is to provide a golf ball with good distance, well-defined spin and greater durability.

15 A further example is Yabuki et al., U.S. Pat. No. 5,716,293 for a Golf Ball which was originally filed in Japan in 1995. Yabuki discloses a golf ball with a rubber solid core containing an oil substance, an oil-resistant coating layer, a wound layer and an ionomer cover layer.

20 Another example is Stanton et al., U.S. Pat. No. 5,836,831 for a Golf Ball, originally filed in 1996. Stanton discloses a liquid filled core having a polyether-amide shell, a wound layer and a polymer cover.

25 There have been many attempts to develop a golf ball that can do everything for every golfer, a golf ball that has tremendous distance, with exceptional feel and outstanding durability. However, current golf balls have been unable to deliver everything.

**BRIEF SUMMARY OF THE INVENTION**

30 The present invention provides a golf ball that has tremendous distance, with exceptional feel and outstanding durability. The present invention is able to accomplish this by providing a four-piece wound golf ball with a polyurethane cover.

35 One aspect of the present invention is a golf ball having a core, a boundary layer, a wound layer and a cover. The boundary layer covers the core and is a thermoplastic material having a Shore D hardness between 40 and 85. The wound layer covers the boundary layer. The cover is preferably a polyurethane material, and it covers the wound layer.

40 Another aspect of the present invention is method for manufacturing a four-piece golf ball. The method includes injection molding a boundary layer over a core. The boundary layer is a thermoplastic material having a Shore D hardness in the range of 40 to 85. The method also includes winding a fiber around the boundary layer to form a wound layer. The method also includes forming a polyurethane layer over the wound layer to form the four-piece golf ball.

45 Yet another aspect of the present invention is a four-piece golf ball having a solid core, a thermoplastic boundary layer, a wound layer and a thermosetting polyurethane cover. The solid core includes a polybutadiene material, has a PGA compression of at least 80, and a diameter in the range of 1.35 inches to 1.58 inches. The boundary layer covers the solid core and is composed of blend of ionomer materials. The boundary layer also has a Shore D hardness between 40 and 85, and a thickness in the range of 0.01 inches to 0.1 inches. The wound layer covers the boundary layer, and has a thickness of 0.05 to 0.1 inches. The thermosetting polyurethane layer covers the wound layer, and has a thickness in the range of 0.01 inches to 0.05 inches.

50 60 65 60 The primary object of the present invention is to provide a golf ball that can deliver exceptional distance with exceptional feel and exceptional durability.

An additional object of the present invention is to provide a golf ball with exceptional distance, exceptional spin around the greens, soft feel for putting and chipping, and an oxygen barrier to prevent degradation of the polybutadiene core over time.

Having briefly described the present invention, the above and further objects, features and advantages thereof will be recognized by those skilled in the pertinent art from the following detailed description of the invention when taken in conjunction with the accompanying drawings.

#### BRIEF DESCRIPTION OF THE SEVERAL VIEWS OF THE DRAWINGS

FIG. 1 is a cross-section view of a four-piece golf ball of the present invention.

FIG. 2 is a cross-sectional view of an alternative embodiment of a four-piece golf ball of the present invention.

#### DETAILED DESCRIPTION OF THE INVENTION

The novel golf ball of the present invention provides greater distance, better feel, and outstanding durability than present golf balls. The present invention is able to achieve this by providing a four-piece golf ball having a high energy core for distance, a boundary layer to prevent degradation of the core, a wound layer for feel and a polyurethane cover for durability.

As illustrated in FIG. 1, the golf ball of the present invention is generally indicated as 10. The golf ball 10 includes a solid core 12, a boundary layer 14, a wound layer 16 and a cover 18. Alternatively, as shown in FIG. 2, the golf ball 10 may include a fluid-filled core 12', a boundary layer 14, a wound layer 16, and a cover 18. The boundary layer 14 that covers the core 12 has a predetermined hardness that is softened by the wound layer 16 and the relatively soft cover 18.

The cover 18 is a polyurethane cover that is relatively soft and has a good durability due to the high resilience of the polyurethane material. The polyurethane cover 18 is composed of a polyurethane material preferably formed from a blend of diisocyanate prepolymers. Preferably, the polyurethane is a thermosetting polyurethane, however, thermoplastic polyurethane materials are within the scope of the present invention. The blend of diisocyanate prepolymers includes at least one TDI-based polyurethane prepolymer and at least one other diisocyanate-based polyurethane prepolymer. In a preferred embodiment, the blend of diisocyanate prepolymers includes at least one PPDI-based polyurethane prepolymer and at least one TDI-based polyurethane prepolymer. Alternative embodiments have a blend which includes at least two different PPDI-based polyurethane prepolymer and at least one TDI-based polyurethane prepolymer. Yet further embodiments may include at least one TDI-based polyurethane prepolymer and at least one MDI-based polyurethane prepolymer. Still further embodiments have only a PPDI-based prepolymer instead of a blend of polyurethane prepolymers. Those skilled in the pertinent art will recognize that multiple variations of diisocyanate prepolymers may be utilized without departing from the scope and spirit of the present invention. The cover 18 is described in greater detail below.

The polyurethane cover 18 encompasses the wound layer 16. The wound layer 16 has a thickness in the range of 0.050 inches to 0.250 inches, preferably in the range of 0.060 inches to 0.150 inches and most preferably in the range of

0.080 to 0.100 inches. A preferred embodiment has a wound layer 16 with a thickness of 0.080 inches. The wound layer 16 is preferably an elastic fiber having a predetermined modulus of elasticity. A preferred elastic fiber is a rubber thread with a cross section of approximately 0.022 inches  $\times$  0.0625 inches, and an ultimate elongation of approximately 1000 grams (the thread has a 1000% elongation under a load of 1000 grams). Devices for winding threads around cores are well known in the golf industry. One such apparatus rotates a golf ball core as it draws thread through a tensioning system from a thread source. The tensioning system usually has several tension wheels for applying tension to the thread during winding around the core. The thread is wound around the core to a predetermined diameter. In constructing the golf ball 10 of the present invention, a similar winding device winds the thread around the boundary layer 14 and core 12.

The wound layer 16 provides a softer feel to the golf ball 10, especially with a solid polybutadiene core 12. The wound layer 16 also provides a golf ball 10 with better spin around the greens while not deterring from the distance performance.

The threads of the wound layer 16 encompass a boundary layer 14, as shown in FIGS. 1 and 2. The boundary layer 14 is preferably composed of a thermoplastic material that has a predetermined hardness. A preferred material for the boundary layer 14 is a blend of ionomers such as those sold by DuPont under the brand name SURLYN® or those sold by Exxon Chemical under the brand name IOTEK®. Alternatively, the boundary layer 14 may be composed of a polyether block amide such as PEBAK®, or a polyester elastomer such as HYTREL®. The boundary layer has a Shore D hardness, as measured by ASTM standards, in range of 55 to 75, preferably 65 to 75, and most preferably 70. The boundary layer 14 is described in greater detail below.

The boundary layer 14 encompasses the core 12. As mentioned above, the core 12 may be solid, hollow, or fluid filled with a liquid or gas. A preferred core 12 is a solid core primarily composed of a polybutadiene material. The fluid filled version of the core 12 is preferably filled with a liquid such as corn syrup or water. The core 12 is described in greater detail below. The most important aspect of the present invention is the novel construction of the golf ball 10. The core 12, boundary layer 14, wound layer 16 and cover 18 construction creates a golf ball 10 that has exceptional overall properties, and has the best performance in many if not all pertinent categories. The positioning of a wound layer 16 over a relatively hard boundary layer 14 with a relatively soft and durable cover 18 creates a unique golf ball 10 that has a good feel and delivers tremendous distance.

As mentioned previously, a preferred material for the cover 18 is a thermosetting polyurethane material. The preferred polyurethane is composed of blend of a TDI-based prepolymer, a second diisocyanate-based polyurethane prepolymer and a curing agent. The TDI-based prepolymer is preferably formed from TDI and a polyether polyol. The second diisocyanate-based polyurethane prepolymer is preferably a PPDI-based prepolymer formed from PPDI and a polyester polyol, preferably a polycaprolactone. The prepolymer blend is cured with a curing agent. The curing agent, or curative, may be a diol (e.g., 1,4 butane diol, trimethylpropanol), a mixture of diols (e.g., 1,4 butane diol and ethylene glycol, or other suitable glycols), a hydroquinone, a mixture of hydroquinones, a triol, a mixture of triols, a diamine, a mixture of diamines, an oligomeric

diamine, a triamine, or a blend of some or all of these materials. Preferably, the curing agent is a blend of a diamine and a mixture of diols.

In an alternative embodiment, the blend of prepolymers includes three diisocyanate-based polyurethane prepolymers. In this embodiment, the TDI-based prepolymer is preferably formed from TDI and a polyether polyol. The second diisocyanate-based polyurethane prepolymer is preferably a PPDI-based prepolymer formed from PPDI and a polyester polyol, preferably a polycaprolactone. The third diisocyanate-based polyurethane prepolymer is a PPDI-based prepolymer formed from PPDI and a polyether polyol. Preferably, the curing agent is a blend of a diamine and a mixture of diols. As mentioned above, alternative embodiments may have variations of the dual blend or the tri-blend, and may use a TDI-based polyurethane prepolymer with other non-PPDI-based polyurethane prepolymers.

Yet another embodiment of a thermosetting polyurethane cover **18** is one that is composed of a single PPDI-based prepolymer instead of a blend. The PPDI-based polyurethane prepolymer provides a polyurethane with a high rebound at a lower hardness, greater durability and improved sound and feel. The PPDI-based prepolymer is preferably cured with a 1,4 butane diol and ethylene glycol mixture. A preferred single PPDI-based prepolymer is a polycaprolactone terminated prepolymer.

The blending of a TDI-based prepolymer with other diisocyanate-based polyurethane prepolymers lowers the viscosity of the mixture, lowers the temperature of the exothermic reaction that occurs when the prepolymers are reacted with the curing agent, and increases the durability. The TDI-based prepolymer may range from 10 to 40 percent of the polyurethane prepolymer blend. Preferably, the TDI-based prepolymer is 30 percent of the polyurethane prepolymer blend. A preferred TDI based prepolymer is a TDI terminated polyether prepolymer available from Uniroyal Chemical Company of Middlebury, Conn., under the trademark ADIPRENE® LF950.

The dual blend and tri-blend formulations will preferably contain a PPDI terminated polyester prepolymer and/or a PPDI terminated polyether prepolymer. A preferred PPDI terminated polyester prepolymer is available from Uniroyal Chemical under the trademark ADIPRENE® LFPX 2950. A preferred PPDI terminated polyether prepolymer is available from Uniroyal Chemical under the trademark ADIPRENE® LFPX 950.

The polyurethane prepolymer blend may have 10 to 40 parts of a TDI terminated polyether prepolymer blended with 60 to 90 parts of a PPDI terminated polyether prepolymer. Alternatively, the polyurethane prepolymer blend may have 10 to 40 parts of a TDI terminated polyether prepolymer blended with 60 to 90 parts of a PPDI terminated polyester prepolymer. Further, the polyurethane prepolymer blend may have 10 to 40 parts of a TDI terminated polyether prepolymer blended with 5 to 90 parts of a PPDI terminated polyether prepolymer and 5 to 90 parts of a PPDI terminated polyester prepolymer. More specific blend formulations are set forth in the Examples below.

The cover **18** of the golf ball **10** of the present invention is most preferably composed of a polyurethane formed from a polyurethane prepolymer blend composed of a TDI-based polyurethane prepolymer and a PPDI-based polyurethane prepolymer, and cured with a mixture of curing agents such as a diamine and a blend of 1,4 butane diol and glycols. A suitable blend of diol and glycols is available from Uniroyal Chemical under the trademark VIBRACURE® A250. A

suitable diamine is toluene ethylene diamine available from Albemarle Corporation of Baton Rouge, La. under the trademark ETHACURE® 100. Other agents which may be utilized during the curing process include dimethylthio-2,4-toluenediamine (such as EHTACURE® 300 available from Albemarle Corporation); trimethyl glycol di-p-aminobenzoate (such as VERSALINK® 740M available from Air Products and Chemicals, Inc., Allentown, Pa.); cyclohexane dimethanol; hydroquinone-bis-hydroxyethyl ether; phenyldiethanol amine mixture (such as VIBRACURE® A93 1 available from Uniroyal Chemical); methylene dianiline sodium chloride complex (such as CAYTOR® 31 available from Uniroyal Chemical); and/or prionene amine. This list of preferred agents (including chain extenders, cross-linkers and curing agents) is not meant to be exhaustive, as any suitable (preferably polyfunctional) chain extender, cross-linker, or curing agent may be used.

The curing agent mixture for the cover **18** of the present invention may have numerous variations. In a preferred embodiment, the curing agent is composed of 30 to 70 parts of a diol blend such as VIBRACURE® 250 to 70 to 30 parts of a diamine such as ETHACURE® 300. Alternatively, the diamine component may be a blend of different diamines such as a blend of EHTACURE® 100 and ETHACURE® 300.

The ratio of the polyurethane prepolymer blend to curing agent is determined by the nitrogen-carbon-oxygen group ("NCO") content of the polyurethane prepolymer blend. For example, the NCO content of the TDI-terminated polyether or TDI-terminated polyester is preferably in the range of 4.0% to 9.0%, while the NCO content of the PPDI-terminated polyether is preferably in the range of 5.0% to 8.0%. The NCO content of the PPDI-terminated polyester is preferably in the range of 2.0% to 6.0%. The NCO content of the polyurethane prepolymer blend ranges from 2% to 8% of the polyurethane prepolymer blend. The amount of curing agent should correspond to 90% to 110% of the mol equivalence of the NCO content of the polyurethane prepolymer blend. The weight ratio of the polyurethane prepolymer blend to the curing agent is preferably in the range of about 10:1 to about 30:1.

Prior to curing, the polyurethane prepolymer blend and curing agent are preferably stored separately. The polyurethane is formed by first heating and mixing the polyurethane prepolymer blend with the curing agent in a mold, and then curing the mixture by applying heat and pressure for a predetermined time period. Additionally, a catalyst (e.g. dibutyl tin dilaurate, a tertiary amine, etc.) may be added to the mixture to expedite the casting process. Specific suitable catalysts include TEDA dissolved in di propylene glycol (such as TEDA L33 available from Witco Corp. Greenwich, Conn., and DABCO 33 LV available from Air Products and Chemicals Inc.) which may be added in amounts of 2-5%, and more preferably TEDA dissolved in 1,4-butane diol which may be added in amounts of 2-5%. Another suitable catalyst includes a blend of 0.5% 33LV or TEDA L33 (above) with 0.1% dibutyl tin dilaurate (available from Witco Corp. or Air Products and Chemicals, Inc.) which is added to a curative such as VIBRACURE® A250. Further, additives such as colorants may also be added to the mixture.

The polyurethane prepolymer blend material is preferably degassed and warmed in a first holding container prior to processing of the cover **18**. The processing temperature for the polyurethane prepolymer blend is preferably in the range of about 100-220° F., and most preferably in the range of about 120-200° F. The polyurethane prepolymer blend is

preferably flowable from the first holding container to a mixing chamber in a range of about 200–1100 grams of material per minute, or as needed for processing. In addition, the polyurethane prepolymer blend material may be agitated in the first holding container, in the range of 0–250 rpm, to maintain a more even distribution of material and to eliminate crystallization.

In the preferred embodiment, the curing agent is a blend of a diamine such as ETHACURE® 300 and a 1,4 butane diol and glycol such as VIBRACURE® A250. As previously mentioned, other curatives may also be utilized in forming the cover 18 of the golf ball 10 of the present invention. The curing agent is preferably degassed and warmed in a second holding container prior to processing of the cover 18. The processing temperature for the curative is preferably in the range of about 50–230° F., and most preferably in the range of about 80–200° F. The curing agent is preferably flowable from the second holding container to the mixing chamber in the range of about 15–75 grams of material per minute, or as needed. If a catalyst is used for processing the cover 18, then the catalyst is added to the curing agent in the second holding container to form a curative mixture. Suitable catalyst are described above. The curing agent and catalyst are agitated, in the range of about 0 to 250 rpm, to maintain an even distribution of catalyst in the curative mixture in the second holding container. It is preferred that the catalyst is added in an amount in the range of about 0.25–5% by weight of the combined polyurethane prepolymer blend and curing agent. Additives may be added to the curative mixture as desired. It was discovered that hydrolytic instability of the polyurethane polymer may be avoided by the addition of a stabilizer such as STABOXYL® (available from Rheinchemie, Trenton, N.J.), in amounts of about 0.25–5% of the polyurethane.

The polyurethane prepolymer blend and curative mixture are preferably added to the common mixing chamber at a temperature in the range of about 160–220° F. A colorant material, such as, for example, titanium dioxide, barium sulfate, and/or zinc oxide in a glycol or castor oil carrier, and/or other additive material(s) as are well known in the art, may be added to the common mixing chamber. The amount of colorant material added is preferably in the range of about 0–10% by weight of the combined polyurethane prepolymer blend and curative materials, and more preferably in the range of about 2–8%. Other additives, such as, for example, polymer fillers, metallic fillers, and/or organic and inorganic fillers (e.g. polymers, balata, ionomers, etc.) may be added as well to increase the specific gravity of the polyurethane cover 18 of the present invention. It was discovered that the addition of barytes (barium sulfate) or a blend of barytes and titanium dioxide (preferably added in a carrier glycol and/or castor oil) to the mixture, in the amounts of about 0.01–30%, may add sufficient weight to the polyurethane cover 18. The added weight to the cover 18 allows for the specific gravity of the core 12 to be lowered thereby allowing for an increased resiliency of the core 12. The entire mixture is preferably agitated in the mixing chamber in the range of about 1 to 250 rpm prior to molding. A more detailed explanation of the process is set forth in this Assignee's co-pending U.S. patent application Ser. No. 09/296,197, entitled Golf Balls And Methods Of Manufacturing The Same, filed on Apr. 20, 1999, which is hereby incorporated by reference in its entirety.

The core 12 of the golf ball 10 is the "engine" for the golf ball 10 such that the inherent properties of the core 12 will strongly determine the initial velocity and distance of the golf ball 10. A higher initial velocity will usually result in a

greater overall distance for a golf ball. In this regard, the Rules of Golf, approved by the United States Golf Association ("USGA") and The Royal and Ancient Golf Club of Saint Andrews, limits the initial velocity of a golf ball to 250 feet (76.2 m) per second (a two percent maximum tolerance allows for an initial velocity of 255 per second) and the overall distance to 280 yards (256 m) plus a six percent tolerance for a total distance of 296.8 yards (the six percent tolerance may be lowered to four percent). A complete description of the Rules of Golf are available on the USGA web page at [www.usga.org](http://www.usga.org). Thus, the initial velocity and overall distance of a golf ball must not exceed these limits in order to conform to the Rules of Golf. Therefore, the core 12 for a USGA approved golf ball is constructed to enable the golf ball 10 to meet, yet not exceed, these limits.

The coefficient of restitution ("COR") is a measure of the resilience of a golf ball. The COR is a measure of the ratio of the relative velocity of the golf ball after direct impact with a hard surface to the relative velocity before impact with the hard surface. The COR may vary from 0 to 1, with 1 equivalent to a completely elastic collision and 0 equivalent to a completely inelastic collision. A golf ball having a COR value closer to 1 will generally correspond to a golf ball having a higher initial velocity and a greater overall distance. The effect of a higher COR value is apparent when a golf club strikes the golf ball 10. The force of the club during a swing is transferred to the golf ball 10. If the golf ball has a high COR (more elastic), then the initial velocity of the golf ball will be greater than if the golf ball had a low COR. In general, a higher compression core will result in a higher COR value.

The core 12 of the golf ball 10 is preferably composed of a blend of a base rubber, a cross-linking agent, a free radical initiator, and one or more fillers or processing aids. A preferred base rubber is a polybutadiene having a cis-1,4 content above 90%, and more preferably 98% or above. A preferred cross-linking agent is a zinc diacrylate, and a commercially available zinc diacrylate is SR-416 from Sartomer Co., Inc., Exton, Pa. Other metal salt di- or mono-(meth)acrylates suitable for use in the present invention include those in which the metal is calcium or magnesium. In the manufacturing process it may be beneficial to pre-mix some cross-linking agent(s), such as, e.g., zinc diacrylate, with the polybutadiene in a master batch prior to blending with other core components.

Free radical initiators are used to promote cross-linking of the base rubber and the cross-linking agent. Suitable free radical initiators for use in the golf ball core 12 of the present invention include peroxides such as dicumyl peroxide, bis-(t-butyl peroxy) diisopropyl benzene, t-butyl perbenzoate, di-t-butyl peroxide, 2,5-dimethyl-2,5-di-5-butylperoxyhexane, 1,1-di (t-butylperoxy) 3,3,5-trimethyl cyclohexane, and the like, all of which are readily commercially available.

Zinc oxide is also preferably included in the core formulation. Zinc oxide may primarily be used as a weight adjusting filler, and is also believed to participate in the cross-linking of the other components of the core (e.g. as a coagent). Additional processing aids such as dispersants and activators may optionally be included. In particular, zinc stearate may be added as a processing aid (e.g. as an activator). Any of a number of specific gravity adjusting fillers may be included to obtain a preferred total weight of the core 12. Examples of such fillers include tungsten and barium sulfate. All such processing aids and fillers are readily commercially available. A particularly useful tungsten filler is WP102 Tungsten (having a 3 micron particle size) available from Atlantic Equipment Engineers (a division of Micron Metals, Inc.), Bergenfield, N.J.

Table 1 below provides the ranges of materials included in the preferred core formulations of the present invention.

TABLE 1

| Core Formulations         |                               |                               |
|---------------------------|-------------------------------|-------------------------------|
| Component                 | Preferred Range               | Most Preferred Range          |
| Polybutadiene             | 100 parts                     | 100 parts                     |
| Zinc diacrylate           | 20-35 phr                     | 25-30 phr                     |
| Zinc oxide                | 0-50 phr                      | 5-15 phr                      |
| Zinc stearate             | 0-15 phr                      | 1-10 phr                      |
| Peroxide                  | 0.2-2.5 phr                   | 0.5-1.5 phr                   |
| Filler<br>(e.g. tungsten) | As desired<br>(e.g. 2-10 phr) | As desired<br>(e.g. 2-10 phr) |

In the present invention, the core components are mixed and compression molded in a conventional manner known to those skilled in the art. The finished core **12** has a diameter of about 1.20 to about 1.64 inches for a golf ball **10** having an outer diameter of 1.68 inches. More preferably, the finished core **12** has a diameter of about 1.30 to about 1.50 inches for a golf ball **10** having an outer diameter of 1.68 inches. Most preferably, the finished core **12** has a diameter of about 1.305 to about 1.345 inches for a golf ball **10** having an outer diameter of 1.68 inches. The core weight is preferably maintained in the range of about 32 to about 40 g. The core PGA compression is preferably maintained in the range of about 55 to 90, and most preferably about 55 to 80.

As used herein, the term "PGA compression" is defined as follows:

$$\text{PGA compression value} = 180 - \text{Riehle compression value}$$

The Riehle compression value is the amount of deformation of a core or a golf ball in inches under a static load of 200 pounds, multiplied by 1000. Accordingly, for a core deformation of 0.110 inches under a load of 200 pounds, the Riehle compression value is 110 and the PGA compression value is 70.

In an alternative embodiment, the core **12** may be hollow or fluid filled. In such an embodiment, as shown in FIG. 2, the core **12** has a shell **12a** encompassing an interior chamber **12b**. The interior chamber may be filled with a fluid **12c**. Exemplary fluids **12c** are water, air, corn syrup, oil, and the like. If a liquid is utilized as the fluid **12c**, then preferably the liquid occupies only half of the volume of the interior chamber **12b**. The compressibility of the fluid is a primary concern in such an embodiment. The shell **12a** should be sufficient to contain the fluid under the tremendous forces exerted on the shell **12a** during impact between a golf club head and the golf ball **10**. A preferred shell **12a** is composed of a polybutadiene material. Alternatively, the shell **12a** may be composed of metal such as titanium, stainless steel or the like. If the fluid **12c** is air, the air may be greater or less than one atmosphere in pressure.

As is described above, the present invention includes at least one boundary layer **14** that is preferably composed of a thermoplastic material or a blend of thermoplastic materials. Most preferably the boundary layer **14** is composed of at least one thermoplastic that contains organic chain molecules and metal ions. The metal ion may be, for example, sodium, zinc, magnesium, lithium, potassium, cesium, or any polar metal ion that serves as a reversible cross-linking site and results in high levels of resilience and impact resistance. Suitable commercially available thermoplastics are ionomers based on ethylene copolymers and containing carboxylic acid groups with metal ions such as described

above. The acid levels in such suitable ionomers may be neutralized to control resiliency, impact resistance and other like properties. In addition, other fillers with ionomer carriers may be used to modify (e.g. preferably increase) the specific gravity of the thermoplastic blend to control the moment of inertia and other like properties. Exemplary commercially available thermoplastic materials suitable for use in a boundary layer **14** of a golf ball **10** of the present invention include, for example, the following materials and/or blends of the following materials: HYTREL® and/or HYLENE® products from DuPont, Wilmington, Del., PEBAX® products from Elf Atochem, Philadelphia, Pa., SURLYN® products from DuPont, and/or ESCOR® or IOTEK® products from Exxon Chemical, Houston, Tex.

The Shore D hardness of the boundary layer **14** is preferably 75. It is preferred that the boundary layer **14** have a hardness of between about 55-85 Shore D. In a preferred embodiment, the boundary layer **14** has a Shore D hardness in the range of about 65-75. One reason for preferring a boundary layer **14** with a Shore D hardness of approximately 75 is to improve the feel of the resultant golf ball. It is also preferred that the boundary layer **14** is composed of a blend of SURLYN® ionomer resins.

SURLYN® 8150, 9150, and 6320 are, respectively, an ionomer resin composed of a sodium neutralized ethylene/methacrylic acid, an ionomer resin composed of a zinc neutralized ethylene/methacrylic acid, and an ionomer resin composed of a terpolymer of ethylene, methacrylic acid and n-butyl acrylate partially neutralized with magnesium, all of which are available from DuPont Polymer Products, Wilmington, Del.

The boundary layer **14** may include a predetermined amount of a baryte mixture. The baryte mixture is included as 8 or 9 parts per hundred parts of the ionomer resins. One preferred baryte mixture is composed of 80% barytes and 20% of an ionomer, and is available from Americhem, Inc., Cuyahoga Falls, Ohio, under the trade designation 38534X1. The Shore D hardness provided in Table 2 below was determined according to ASTM D2240.

Table 2 below sets forth physical data for suitable boundary layers **14** that were manufactured and incorporated into specific examples. As is shown in Table 2 below, each of the boundary layers **14** were composed of an ionomer blend and the specific percentages are provided. The thickness of each of the boundary layers **14** varies from 0.0525 and 0.058 inches. The Shore D hardness varies between 58 and 65, however, those skilled in the relevant art will recognize that materials for the boundary layer **14** with higher Shore D hardness values are conventional and within the scope of the invention.

TABLE 2

| Ex. | SURLYN ® |        |        | Thickness<br>(inches) | Shore D<br>Hardness |
|-----|----------|--------|--------|-----------------------|---------------------|
|     | No.      | % 8150 | % 9150 | % 6320                |                     |
| 1   | 40       | 40     | 20     | 0.058                 | 58                  |
| 2   | 45       | 45     | 10     | 0.0525                | 62                  |
| 3   | 45       | 45     | 10     | 0.0525                | 62                  |
| 4   | 40       | 40     | 20     | 0.058                 | 60                  |
| 5   | 40       | 40     | 20     | 0.058                 | 60                  |
| 6   | 40       | 40     | 20     | 0.058                 | 60                  |
| 7   | 45       | 45     | 20     | 0.0525                | 62                  |
| 8   | 45       | 45     | 20     | 0.0525                | 62                  |
| 9   | 50       | 50     | 0      | 0.0525                | 65                  |

TABLE 2-continued

| Ex. | SURLYN ® |        |        | Thickness | Shore D  |
|-----|----------|--------|--------|-----------|----------|
| No. | % 8150   | % 9150 | % 6320 | (inches)  | Hardness |
| 10  | 45       | 45     | 10     | 0.0525    | 62       |
| 11  | 45       | 45     | 10     | 0.0525    | 62       |
| 12  | 45       | 45     | 10     | 0.0525    | 62       |

TABLE 3

| Ex. | Polyurethane prepolymer |        |        |        |        | Thickness | Shore D  |
|-----|-------------------------|--------|--------|--------|--------|-----------|----------|
| No. | TDI                     | PPDI-1 | PPDI-2 | PPDI-3 | PPDI-4 | (inches)  | Hardness |
| 1   | 30                      | 70     |        |        |        | 0.0375    | 47       |
| 2   | 30                      |        | 20     | 50     |        | 0.0300    | 53       |
| 3   | 30                      |        |        |        | 70     | 0.0300    | 47       |
| 4   | 30                      |        |        |        | 70     | 0.0375    | 47       |
| 5   | 30                      | 50     | 20     |        |        | 0.0375    | 47       |
| 6   | 30                      |        |        |        | 70     | 0.0375    | 47       |
| 7   | 30                      | 50     | 20     |        |        | 0.0300    | 47       |
| 8   | 30                      |        | 20     | 50     |        | 0.0300    | 53       |
| 9   | 30                      | 70     |        |        |        | 0.0300    | 53       |
| 10  | 20                      | 80     |        |        |        | 0.0300    | 47       |
| 11  | 30                      | 70     |        |        |        | 0.0300    | 47       |
| 12  | 30                      | 70     |        |        |        | 0.0300    | 47       |

Table 3 sets forth the properties of the exemplary cover layers 18. The number of parts of each polyurethane prepolymer for each of the cover layers 18 is provided in columns 2 through 6. Column 2 includes the number of parts of the TDI-terminated polyether prepolymer, ADIPRENE® LF950. Column 3 includes the number of parts of the PPDI terminated polyether prepolymer, ADIPRENE® LFPX950. Column 4 includes the number of parts of the PPDI terminated polyester (polycaprolactone) prepolymer, ADIPRENE® LFPX2950. Column 5 includes the number of parts of the PPDI terminated polyether prepolymer, ADIPRENE® LFPX590. The difference between LFPX590 and LFPX950 is the NCO content and the molecular weight of the polyol (ether) backbone, with LFPX950 having a NCO content in the range of approximately 5.45% to approximately 5.75%, and LFPX590 having a NCO content in the range of approximately 5.6% to approximately 6.2%. Column 6 includes the number of parts of the PPDI terminated polyester (polycaprolactone) prepolymer, ADIPRENE® LFPX2952. The difference between LFPX2950 and LFPX2952 is the NCO content, with LFPX2950 having a NCO content in the range of approximately 3.55% to approximately 3.85%, and LFPX2952 having a NCO content in the range of approximately 4.45% to approximately 5.05%. Each of the polyurethane prepolymer blends for examples 1-9 and 11-12 were cured with a blend of curing agents. The blend of curing agents was composed of 50 parts ETHACURE 300 (a diamine curing agent) and 50 parts VIBRACURE A250 (a blend of a 1,4 butane diol and glycol). Example 10 of the golf balls 10 of the present invention was cured with a blend of 70 parts ETHACURE 300 and 30 parts VIBRACURE A250. The thickness of the exemplary covers 18 is either 0.0300 inches or 0.0375 inches. The Shore D hardness of the exemplary cover layer 18 is either 47 degrees or 53 degrees.

From the foregoing it is believed that those skilled in the pertinent art will recognize the meritorious advancement of this invention and will readily understand that while the present invention has been described in association with a preferred embodiment thereof, and other embodiments illustrated in the accompanying drawings, numerous changes, modifications and substitutions of equivalents may be made therein without departing from the spirit and scope of this invention which is intended to be unlimited by the foregoing except as may appear in the following appended claims. Therefore, the embodiments of the invention in which an exclusive property or privilege is claimed are defined in the following appended claims.

I claim as my invention:

1. A golf ball comprising:

a hollow core having a diameter ranging from 1.30 inches to 1.50 inches;

a boundary layer covering the core, the boundary layer formed from a blend of ionomer materials consisting of 40, 45, or 50 parts of an ionomer resin composed of sodium neutralized ethylene/methacrylic acid, 40, 45 or 50 parts of an ionomer resin composed of a zinc neutralized ethylene/methacrylic acid, and 0,10, or 20 parts of an ionomer resin composed of a terpolymer of ethylene, methacrylic acid and n-butyl acrylate partially neutralized with magnesium, having a Shore D hardness between 58 to 65 and a thickness in the range of 0.0525 inch to 0.58 inch;

a wound layer covering the boundary layer, the wound layer having a thickness of 0.06 inch to 0.150 inch; and a cover comprising a thermoset polyurethane material covering the wound layer, the cover having a thickness ranging from 0.030 inch to 0.0375 inch.

2. A golf ball comprising:

a solid core comprising a polybutadiene material, having a PGA compression of 55 to 80, a weight of 32 grams to 40 grams, and a diameter in the range of 1.30 inches to 1.50 inches;

a boundary layer covering the solid core, the boundary layer formed from a blend of ionomer materials consisting of 40, 45, or 50 parts of an ionomer resin composed of sodium neutralized ethylene/methacrylic acid, 40, 45, or 50 parts of an ionomer resin composed of a zinc neutralized ethylene/methacrylic acid, and 0,10, or 20 parts of an ionomer resin composed of a terpolymer of ethylene, methacrylic acid and n-butyl acrylate partially neutralized with magnesium, having a Shore D hardness between 58 to 65 and a thickness in the range of 0.0525 inch to 0.58 inch;

a wound layer covering the boundary layer, the wound layer having a thickness of 0.06 inch to 0.150 inch; and a thermosetting polyurethane layer covering the wound layer, the thermosetting polyurethane layer having a thickness in the range of 0.01 inch to 0.05 inch.

\* \* \* \* \*